

G. A. HENDERSON AND H. K. STEPHENSON,  
PAVEMENT AND PROCESS FOR MAKING THE SAME,  
APPLICATION FILED APR. 15, 1920. RENEWED JAN. 4, 1922.

1,409,104.

Patented Mar. 7, 1922.

2 SHEETS—SHEET 1.



Witnesses:  
L. J. White  
C. H. Gerke

Inventors: George Stephenson  
H. H. Stephenson, by G. Stephenson, attorney

G. A. HENDERSON AND H. K. STEPHENSON.  
PAVEMENT AND PROCESS FOR MAKING THE SAME.  
APPLICATION FILED APR. 15, 1920. RENEWED JAN. 4, 1922.

1,409,104.

Patented Mar. 7, 1922.

2 SHEETS—SHEET 2.

Fig. 2.



Fig. 3.



Witnesses:  
L. J. White  
Ed. Jones

Inventors:  
George Henderson  
H. K. Stephenson, by G. Henderson,  
Attorneys

# UNITED STATES PATENT OFFICE.

GEORGE A. HENDERSON AND HENSON K. STEPHENSON, OF ST. ALBANS, WEST VIRGINIA, ASSIGNORS TO THE INTERNATIONAL BITUCONCRETE COMPANY, A CORPORATION OF DELAWARE.

## PAVEMENT AND PROCESS FOR MAKING THE SAME.

1,409,104.

Specification of Letters Patent.

Patented Mar. 7, 1922.

Application filed April 15, 1920, Serial No. 374,078. Renewed January 4, 1922. Serial No. 527,056.

*To all whom it may concern:*

Be it known that we, GEORGE A. HENDERSON and HENSON K. STEPHENSON, both citizens of the United States, residing at St. 5 Albans, in the county of Kanawha and State of West Virginia, (whose post-office address is St. Albans, West Virginia,) have invented new and useful Improvements in Pavements and Processes for Making the Same, of 10 which the following is a specification.

The invention relates to improvements in compositions for paving and like structures in which pitch is used as the impregnating and cementing agency of vegetable and mineral matter, and the object of the invention 15 is to produce inherent stability and density of such products as are described in the said Henderson's United States Patent No. 1,040,321 of Oct. 8, 1912, and his co-pending 20 application for Letters Patent, Serial Number 212,194 of 1918, for pavements and process for making the same.

The invention will be best understood by reference to the accompanying drawings, it 25 being premised that various changes may be made in the apparatus within the scope of the appended claims. Fig. 1 is a side elevation partly in section, Fig. 2 a cross section and Fig. 3 an end view of apparatus adaptable to the process. Fig. 4 is a detail, sectional view of a compression die; in which drawings A represents the frame work supporting the machine, C a furnace, D an asphalt heating tank heated by the furnace, 30 within the lines of which tank are rigidly hung an impregnating drum (I), H a screw conveyor and its housing, G an aggregate chamber, F a dust hopper, F<sup>2</sup> a gate valve to chute F<sup>2</sup> to drum I in which all of the 35 ingredients are agitated under indirect heat supplied by the heated bitumen in tank D partially surrounding the drum I, and by direct heat sucked from the furnace C therethrough by exhaust K and then discharged 40 in a continuous flow of material under pressure through drum-mouth L into vacuum chamber M, all for the purposes hereinafter described.

In carrying out the invention fibrous particles, preferably that "spent hard wood" described in said Patent 1,040,321, but while containing water in lieu of sap and cellular tissue removed therefrom, are subjected to the action of bicarbonate of soda in solution to

neutralize any remaining pyroligneous acids 55 of such woody particles. These woody particles are then only partially dried while being heated and agitated under the influence of suction in said drum I until their moisture content is reduced to approximately 20% of their solid volume. In this operation the wood dust, when sufficiently dry to float in air suspension, is sucked out of the drum by exhaust K before such dust becomes hydro-carbon, and the clean, partially dried 60 woody particles are then taken from the vat, bagged, and weighed in predetermined quantity for use in the process as herein-after described.

It has been heretofore proposed to mix in 70 excess of fifty per cent. by weight of truly impalpable dust of earthy nature with a bituminous compound of relatively soft consistency, as tested for penetration, viz., approximately 100-120 penetration, which bituminous compound is more of a lubricant 75 permeating such dust than it is a binder such as the heavier bituminous compound of approximately 40-50 penetration used in the so-called "mixing-method" of producing 80 paving structures, as distinguished from the "penetration method" both known to the trade and prior art. In order to practically agglomerate in colloidal suspension such substantial proportion of impalpable mineral dust in such a heavy bituminous binder, 85 to act as a filler of voids between, (as distinguished from pores within) particles of larger aggregate sought to be bound thereby, we preliminarily prepare a mixture of such 90 dust of colloidal nature, and of from 5% to 20% pulverized sulfur,  $\frac{1}{2}$  of 1% to 4% sodium chloride, and from  $\frac{1}{2}$  of 1% to 3% of sulfate of copper, in proportions in relation to the final product constituents herein- 95 after described, and inject this mixture in air suspension, under the influence of heat and suction, into a mixture of larger mineral and vegetable aggregate, while agitating the same in a drum, (I), during dehydration of 100 that mass in the presence of molten bitumen. We have discovered that by this means we obtain temporary fluidity of the bituminous cement and substantial ebullition of the mass, the steam there and then evolved acting as 105 the carrying agent to perfectly agglomerate the bituminous cement uniformly throughout the aggregate and to aid in colloidally

suspending the dust therein, and facilitating chemical combination and vulcanization of the ingredients.

Depending on the nature of the product of our process, as regards its consistency, degree of hardness and of elasticity, the proportions of dust and chemicals are varied. In example, to provide a mastic filler as a matrix within interstices of larger metal of 10 a macadam highway, we prefer the following proportions: the final product shall contain bitumen containing by weight the derivative of one per cent. sodium chloride, copper sulfate one per cent., sulfur five per cent. and 15 93% pitch cement or bitumen, known to the trade, and the product of this process shall contain, in example, 30% of sulpho-chlorinated bitumen, 30% impalpable mineral dust, 20% woody particles freed from vegetable dust as in the above manner described, and 20% larger mineral aggregate composed of crushed stone, slag or gravel, containing all dust of fracture, representing in approximate volume the following proportions: 20 viz., of bituminous compound 36%, impalpable dust 20%, vegetable particles, in the absence of dust, 32%, mineral aggregate 12%. In our use of kieselguhr or other light weight impalpable mineral dust, the volume 25 percentages shall be identical with the above, with corresponding changes in proportions by weight.

In operation of said apparatus the vegetable particles, in the absence of dust, are 30 deposited in predetermined measured proportion in mixer E simultaneously with the depositing therein of the predetermined measured quantity of pitch heated to fluidity in tank D, by heat in furnace C supplied 40 by burners C' with oil under air pressure through supply pipe C<sup>2</sup> from a fuel oil tank carried on traction unit forward of the plant, not shown in the drawings.

Tank D is initially charged from an 45 auxiliary supply, with heated bitumen, through inlet pipe D'. By operating three-way cock D<sup>2</sup> the heated bitumen is sucked through pump X, cock D<sup>4</sup> and pipe D<sup>3</sup> to tank D. When charged with hot bitumen 50 the supply to tank D is shut off by closing the inlet through cock D<sup>2</sup>, in pipe D', which operation opens suction through pipe D<sup>5</sup> and the pump then operates to suck the heated bitumen up from the bottom of the tank D 55 on one side of drum I and to deposit it at the top of tank D on the reverse side of drum I, which action is designed to (a) furnish a ready supply of heated bitumen through cock D<sup>4</sup> manually operated to 60 charge pitch weigh-bucket, not shown, for depositing the measured quantity of pitch into mixer E, and (b) to cause continuous agitation of the heating bitumen in tank D, to prevent coking of the mass therein.

65 The pitch in excessive quantity in rela-

tion to the woody particles in mixer E, at this stage of the process, is first mixed with said woody particles in mixer E and the mineral aggregate is then measured thereinto, and these three ingredients then 70 agitated in the presence of an excess of pitch, or more than would be required in the final product if such excess were not taken up by the added dust in the manner hereinafter described, by the action of interdigitating blades E', E' anchored to reciprocating shafts E<sup>2</sup>, E<sup>3</sup> revolved in the same direction as each other by cog E<sup>6</sup> on driven shaft E<sup>3</sup> (Fig. 3) operating cogs E<sup>6</sup>, E<sup>7</sup> bearing the blades E<sup>1</sup>, E<sup>1</sup> (Fig. 1) aforesaid, 75 connected through driven shaft E<sup>3</sup> with the motive power P in the manner shown.

When the three ingredients just mentioned have been mixed in mixer E one minute, and after each particle of the mineral and 80 the vegetable aggregate has been coated with the pitch, the mass is dumped, by manual operation of lever L' (Fig. 1) designed to open the bottom of pug mixer L, in halves, E<sup>9</sup>, E<sup>9</sup> (Fig. 2) (as per known construction,) into aggregate chamber G subjected 85 to suction through pipe G' to exhauster K', whereupon the operation in mixer E is repeated.

Simultaneously with the above mixing operation, the aforesaid dust mixed with chemicals, is, in predetermined measured quantity, deposited in hopper F, from which it is gradually fed to chute F<sup>2</sup> through gate-valve F<sup>3</sup> operated by cogged connection F<sup>5</sup> 100 meshing with cog F<sup>6</sup> on driven shaft L<sup>3</sup>, and the dust is precipitated by gravity through chute F<sup>2</sup> in continuous flow to the entrance to drum I at the point shown in Fig. 1 as I<sup>3</sup>. At this point the hot air and fumes from the furnace C are sucked 105 into the drum I, carrying said dust thereinto in air suspension by the operation of exhauster K. The number of revolutions per minute of gate-valve F<sup>3</sup> is fixed consistent with the capacity of the entire machine and its connections with driven central shaft I<sup>4</sup> (Fig. 1) and motive power P. 110

It is designed that the excess pitch in preliminary mixer E shall be partially taken 115 up by the mineral aggregate therein added, and finally such excess exhausted by the addition of the dust in drum I in the manner above described, so that in the final product the proper percentages of each of the ingredients may be present.

The housing of screw conveyor H forms the bottom of chamber G and that conveyor is designed to be revolved at a speed consistent with the object to move the contents 120 of chamber G, viz., one batch of ingredients from mixer E from chamber G the length of conveyor E within five minutes time, the mixing operation in mixer E being repeatedly completed every five minutes in- 125 130

cluding the time in which the ingredients are mixing therein, and that time required for dumping mixer E to chamber G, thus providing a continuous flow of mixed and measured ingredients to drum I, for the purpose of providing a continuous flow of material out of drum I into vacuum discharge chamber M.

The period of agitation within drum I is fixed by the speed of the central shaft I<sup>4</sup>, and its blades I<sup>7</sup>, driven by chain I<sup>5</sup> and pulley I<sup>6</sup> connected with the motive power P, and by the number, inclination and dimensions of agitating blades I<sup>7</sup> anchored to the central shaft by sleeves I<sup>8</sup>, which blades are set at such an angle to the central shaft to form a perfect screw in their operation to move the mass in drum I the entire length of the drum within five minutes. During this period the mass is subjected to agitation, and to such suction by exhaust K as to produce a partial vacuum within drum I, equivalent to approximately two thirds atmospheric, viz., 466 barometric pressure, at which pressure the boiling point of water (that residual moisture within the aggregate then being dehydrated) requires a temperature of not exceeding 88 C. (190 deg. Fahr.) as compared with 100 deg. C. (212 deg. Fahr.) at atmospheric pressure. In this connection we have discovered that such reduced pressure within the mass inclosure I aids in its ebullition, as and for the purpose herein-after described, namely:

The exact temperature of the mass within drum I is essential to be uniformly fixed and registered for the purposes of this process, and this we accomplish by regulating the degree of heat of the bitumen in tank D, by manually fixing the degree of pressure and quantity of oil supply to the burners C<sup>1</sup>, which burners indirectly heat, through the bitumen in tank D, the contents of mixer E, conveyor H, and drum I in the manner shown in Fig. 1. The heat in drum I is further regulated by manually adjusting sliding valve I<sup>2</sup> (Fig. 1.) through which valve air of atmospheric temperature is admitted and mixed with that hot air from the furnace C. The temperature of the mass in drum I, thus fixed, is registered by a hand thermometer as it emerges from drum I, and by the use of fixed thermometers set within the lines of drum I and tank D respectively, at the points shown in Fig. 1 at T<sup>1</sup> T<sup>2</sup>.

When in drum I extreme fluidity of the mass (producing a honey-combed effect) is caused by steam in evolution from said residual moisture, escaping from the pores of the woody particles, abnormally enlarging the pores thereof, and entrapping the bituminous cement therein, under the influences of said suction and heat, agitation of the mass, and instantaneous action of the chemicals introduced thereto in air suspen-

sion with the dust, which action perfectly disseminates the bitumen throughout the mass and entraps the dust therein while the bitumen is in a state of momentary ebullition sufficient in time and extent for the designed purpose, viz., the colloidal suspension of dust in the bitumen. When the mass is completely dehydrated in this manner, the chemicals are married in a combined state with the bitumen, at which time the ebullition at once subsides.

The mass in drum I in completing its passage therethrough is subjected to slight compression by the action of blades I<sup>7</sup>, which compact the same through drum mouth L. This compacting aids in the removal of residual gas and air bubbles from the hot mass, by its suction to the atmosphere through exhaust K.

In the above operation the impalpable particles of dust are separated from their neighboring particles of dust by the thinnest possible film of the heavy bituminous compound (as distinguished from that bituminous binder composed of sulfur and bitumen such as described in Henderson's United States Patents Numbers 1,264,932 and 1,266,261 of 1918.) The combination of the said chemicals with the bitumen, and the entrapping therein in colloidal suspension of said substantial quantity of impalpable mineral matter, is due, in our opinion, to the means herein disclosed, of providing said temporary fluidity of the bituminous ingredient, (viz., said thin films forming a honey-combing effect) which, nevertheless, sets to density and afterwards hardens in the final product to the extent of the predetermined quantity of said dust and chemicals, within the said limits, present in the operation.

Chamber M (Fig. 1) is continuously closed at its mouth and discharge end by the material pressed through them. The action of exhaust K, connected therewith by exhaust stack M', produces within chamber M partial vacuum to-wit: that equivalent to a barometric pressure of 152 mm. or approximately one-fifth normal atmospheric pressure. This condition, in conjunction with the means for compacting the material in chamber M, is designed to free it from any residual gas or air preliminary to final compaction of the mass in the manner herein-after described. In chamber M the shaft of screw conveyor M<sup>3</sup>, driven by the machine's motive power by connection M<sup>4</sup>, as shown, is operated horizontally whereas the bottom of chamber M is constructed so as to provide an upward grade of approximately ten per cent. toward the compression die Y. The conveyor M<sup>3</sup> converges in its pitch in ratio corresponding to its incline, up which the material is forced by the revolutions of the conveyor, thus providing, as we have demon-

strated in practice, sufficient resistance to the onward movement of the plastic material in the chamber M toward and through die Y to effect substantial compression of the material in chamber M before it reaches the die, to entirely free it of its residual air and gas content within the vacuum influence in chamber M provided. In this manner we avoid the entrapping of air and gas in the mass when finally compacted in moulds or otherwise, and inherent stability and density of our product is increased over that of the prior art in this manner.

The degree of compression to be applied to our product of this process is fixed by the dimensions of the die Y in relation to the power applied to compact the material through it. After emerging from the die in a continuous flow the hot, plastic material is compacted in moulds to shape, or when used as a matrix to fill the voids between the larger stone of macadam highway, in example, as described in the applicant Henderson's co-pending application Serial Number 212,194, of 1918, the material consisting of said denatured hard wood chips, impregnated with bitumen in the absence of wood dust, mixed with larger mineral aggregate precoated with bitumen, and filled with bitumen, colloidally suspending mineral dust chemically treated in the manner hereinabove described, is spread over and compacted within the interstices of larger mineral aggregate, in situ, on a highway, in the following manner, illustrated in Fig. 1:

Multipedal units C<sup>3</sup>, C<sup>3</sup>, passing around and meshing with cogged drums C<sup>4</sup>, bearing axles C<sup>5</sup>, C<sup>6</sup> operate independently of each other to support the machine by connection with its frame work A, in its course forward; and constitute the sides of furnace C to prevent lateral suction of outside air to the furnace C. The ends of furnace C are composed of heavy leather strips C<sup>6</sup>, C<sup>6</sup>, inserted in steel members to scrape over the road's surface, for like purpose. Scarifiers B suitably attached to the frame work of the machine, by resilient members, not shown, (but known to the trade) are designed to plow the road for a depth of from two to three inches, and to loosen the stone aggregate thereof. Suction through furnace C, caused by the operation of exhauster K, is designed to suck up from the interstices and surface of the road, such dust as may be loosened from its aggregate by the scarifiers in combination with the blasts of flame and air, under pressure, from burners C', C', directed onto said road; and to deposit said dust, in air suspension, into drum I in a continuous operation during the above described process in which additional dust, containing the aforesaid chemicals, is likewise carried in air suspension within drum I. We have discovered in practice that,

within relatively close limits, the quantity of dust removable from the road itself, is sufficient to produce the desired density of our product when added to that dust injected to the mass through chute F<sup>2</sup>. In practice we 70 specify and incorporate in the mass considerably more dust than is required to fill all voids between the larger particles when such dust is colloidally suspended in the bituminous compound; and have discovered that 75 when such an excess of this mixture is present the stability and density of the product is correspondingly increased.

The dust-cleared, loose stone of the highway, heated by said flame-blasts in the course 80 of the machine over it, is then coated with preheated bitumen from an auxiliary supply within a traction unit (not shown), through bitumen supply pipe O and said heated bitumen is forced through pipe O by air compression, to rotary penetration nozzles O' at the rear of the machine, into the interstices of the scarified surface. As the machine passes over this surface the matrix of the process hereinabove described, is chuted to 90 place thereover in quantity approximately one inch in thickness, manually raked to shape and compacted into the open, dust-cleared, bituminized interstices of the heated stone in situ.

We claim:

1. The herein described process which consists in mixing moist vegetable particles in the absence of vegetable dust with an excess of bitumen preheated to a temperature 100 above the boiling point of the moisture; then mixing therewith mineral aggregate in relatively large sizes; then agitating the mass in a vat subjected to suction under the influence of sufficient applied heat to completely dehydrate the same while gradually introducing in air suspension and entrapping therein impalpable mineral dust pre-mixed with sulfur, sodium chloride and copper sulfate, in quantity sufficient to adsorb 110 the excess bitumen; then subjecting the mass to heat and pressure in partial vacuo and compacting the same to shape.

2. The herein described process of treating a metal highway consisting in mixing 115 and dehydrating mineral and vegetable aggregate in the presence of an excess of pure bituminous binder in a vat under the influence of sustained heat and suction sufficient for the purpose, while adding thereto 120 in air suspension impalpable dust sucked therein from interstitial spaces of the highway created by scarifying the same, and blowing flame and air there into, simultaneously depositing in air suspension within 125 said vat additional dust mixed with sodium chloride, copper sulfate and sulfur sufficient in quantity to adsorb the excess bituminous binder, heating said scarified metal of the highway and causing a bituminous com- 130

pound to penetrate the same in its dustless, loose, heated condition; then spreading said mixed material thereover and compacting the same to shape.

5 3. A bituminous composition comprising mineral and vegetable matter impregnated and coated in the absence of dust with a bituminous binder, the interstices between which matter representing at least forty per 10 cent, by volume of the final product, being completely filled with a matrix of mineral dust colloidally suspended in sulfochlorinated bitumen.

4. A paving structure consisting of a broken stone base of relative large sizes of stone 15 coated with a pure bituminous binder the

interstices between which are filled with mineral and vegetable matter of smaller sizes impregnated and coated in the absence of dust with bitumen the interstices between 20 which are filled with a mastic of impalpable mineral dust colloidally suspended in sulfochlorinated bitumen.

In witness whereof we have hereunto set our hands in the presence of two witnesses 25 this 30th day of March, 1920.

GEORGE A. HENDERSON.  
HENSON K. STEPHENSON.

In the presence of—

L. J. WHITE,  
C. H. ZERKEE.